



US005477610A

**United States Patent** [19]**Sawada et al.**[11] **Patent Number:** **5,477,610**[45] **Date of Patent:** **Dec. 26, 1995**

[54] **METHOD OF MANUFACTURING  
COMPOSITE CONDUCTOR HAVING HEAT  
RESISTANCE OR OXIDATION RESISTANCE**

2,975,078 3/1961 Rayfield .  
3,109,053 10/1963 Ahearn .  
3,636,242 1/1972 Hansson .  
4,189,331 2/1980 Roy ..... 148/6.31  
4,620,086 10/1986 Ades et al. .  
4,707,416 11/1987 Ebata et al. .  
5,035,957 7/1991 Bartlett et al. .

[75] Inventors: **Kazuo Sawada; Shinji Inazawa;  
Kouichi Yamada**, all of Osaka, Japan

[73] Assignee: **Sumitomo Electric Industries, Ltd.,**  
Osaka, Japan

[21] Appl. No.: **210,624**

[22] Filed: **Mar. 18, 1994**

**Related U.S. Application Data**

[62] Division of Ser. No. 185,276, Jan. 24, 1994, Pat. No. 5,443,905, which is a continuation of Ser. No. 823,995, Jan. 22, 1992, abandoned.

**Foreign Application Priority Data**

Jan. 24, 1991 [JP] Japan ..... 3-7269

[51] **Int. Cl.<sup>6</sup>** ..... **H01B 13/20**

[52] **U.S. Cl.** ..... **29/828; 427/117; 427/118;  
427/356**

[58] **Field of Search** ..... **427/117, 118,  
427/356; 428/698, 697, 469, 699, 368;  
174/126.1, 126.2; 29/828**

**References Cited****U.S. PATENT DOCUMENTS**

2,207,579 7/1940 Carl .

**FOREIGN PATENT DOCUMENTS**

0029888 6/1981 European Pat. Off. .  
0170440 2/1986 European Pat. Off. .  
0179527A1 4/1986 European Pat. Off. .

*Primary Examiner*—Roy V. King  
*Attorney, Agent, or Firm*—W. G. Fasse; W. F. Fasse

**[57] ABSTRACT**

A method is provided for manufacturing a composite conductor having a copper or copper alloy core, a conductive ceramic intermediate layer and a nickel outer layer, and being suitable for high temperature applications. The method involves first preparing the copper or copper alloy core, then extruding a mixture of conductive ceramic powder and a binder around the core to form the ceramic layer, and then applying a nickel tape as an outer covering. As further steps, a seam of the nickel tape covering is welded, the product is passed through a cladding die, and finally the product is drawn to form the desired conductor with a preselected diameter. Optionally, a further ceramic layer can be applied around the nickel layer.

**7 Claims, 1 Drawing Sheet**

FIG. 1



FIG. 2



## 1

**METHOD OF MANUFACTURING  
COMPOSITE CONDUCTOR HAVING HEAT  
RESISTANCE OR OXIDATION RESISTANCE**

**CROSS-REFERENCE TO RELATED  
APPLICATIONS**

This is a Divisional of U.S. patent application Ser. No. 08/185,276, filed Jan. 24, 1994 (now U.S. Pat. No. 5,443,905, issue date Aug. 22, 1995), which in turn is a continuation of U.S. patent application Ser. No. 07/823,995, filed Jan. 22, 1992 (now abandoned).

**FIELD OF THE INVENTION**

The present invention relates to an electric conductor, which can be used under a high temperature and/or in an oxidizing atmosphere.

**BACKGROUND INFORMATION**

An electric conductor is generally made of aluminum, an aluminum alloy, copper or a copper alloy. However, aluminum has a low melting point of 660° C. and exhibits no strength under a high temperature. An aluminum alloy also has similar problems. On the other hand, copper has a melting point of 1063° C. and is superior to aluminum in strength under a high temperature.

However, copper is easily oxidized under a high temperature. A copper alloy also has a similar problem. Thus, a heat-resistant conductor is formed by a nickel-plated copper wire which is made of copper having a nickel-plated surface.

However, although such a nickel-plated copper wire causes no problem when the same is used at about 400° C., its conductive property is reduced under a higher temperature due to diffusion and alloying of copper and nickel. When the wire is used at 600° C. for 2000 hours, for example, its conductivity is reduced by about 20%. While platinum and gold have no such problem, it is inadvisable to put these materials into practice since the same are extremely high-priced.

**SUMMARY OF THE INVENTION**

It is an object of the present invention to solve the above problem of the prior art and provide a low cost highly conductive conductor, whose conductivity is not reduced under a high temperature.

A composite conductor according to the present invention comprises a core which is made of copper or a copper alloy, a conductive ceramics layer which is provided around the core, and a nickel layer which is provided on the exterior of the conductive ceramics layer.

In order to prevent the nickel layer from oxidation under a high temperature, an oxidation inhibiting ceramics layer may be further provided on the exterior of the nickel layer.

The present composite conductor can be manufactured by the following method, for example: Namely coating a core material by extruding a mixture of conductive ceramics powder and a binder around the core material for forming a conductive ceramics layer on the core, then covering the conductive ceramics coated core with a nickel tape under an atmosphere of an inert gas or a reducing gas, continuously welding a seam of the nickel tape and cladding the wire by a cladding die, and then drawing the clad wire to a prescribed wire diameter.

## 2

When a ceramics layer is further provided around the nickel layer in order to prevent the same from oxidation or the like, this layer can be formed around the drawn wire.

In the composite conductor according to the present invention, the core is made of copper or a copper alloy. Copper or a copper alloy, having the highest conductivity next to silver, is relatively low-priced as compared with silver, and industrially available. Thus, the present composite conductor comprising a core of copper or a copper alloy can be manufactured at a low cost for industrial purposes.

It is possible to improve the strength of the conductor under a high temperature without substantially reducing the conductivity, by employing a copper alloy containing 0.1% of silver.

According to the present invention, the electrically conducting ceramics layer may be made of a carbide, a nitride, a boride or a silicide of a transition metal such as tungsten carbide, zirconium nitride, titanium boride or molybdenum silicide, or carbon, molybdenum disulfide or the like.

According to the present invention, the electrically conducting ceramics layer which is provided between the core part and the nickel layer prevents diffusion from the core to the nickel layer and vice versa under a high temperature. According to the present invention, therefore, the conductivity is not reduced even if the conductor is used for a long time in a high-temperature oxidizing atmosphere.

The electrically conducting ceramics layer has preferably a thickness of at least 0.05 μm. Further, particles forming the ceramics layer are preferably not more than 5 μm in mean particle diameter.

In an oxidizing atmosphere of at least 500° C., oxidation of nickel may not be negligible and hence it is preferable to provide an oxidation inhibiting outer ceramics layer in this case, in order to prevent oxidation of the nickel layer. For the purpose of preventing oxidation, the outer ceramics layer is preferably at least 0.3 μm in thickness. In order to provide sufficient insulability, it is preferable to employ insulating ceramics in the outer oxidation inhibiting ceramics layer having a thickness of at least 1 μm.

The foregoing and other objects, features, aspects and advantages of the present invention will become more apparent from the following detailed description of the present invention when taken in conjunction with the accompanying drawings.

**BRIEF DESCRIPTION OF THE DRAWINGS**

FIG. 1 is a sectional view showing a composite conductor according to an embodiment of the present invention. Referring to FIG. 1, a conductive ceramics layer 2 is provided around a core 1 of copper or a copper alloy, and a nickel layer 3 is provided around the conductive ceramics layer; and

FIG. 2 is a sectional view showing a composite conductor according to another embodiment of the present invention. Referring to FIG. 2, an oxidation inhibiting ceramics layer 4 is further provided around the nickel layer 3.

**DESCRIPTION OF THE PREFERRED  
EMBODIMENTS**

**EXAMPLE 1 OF THE INVENTION**

A continuously supplied copper wire having a diameter of 2.8 mm was degreased and washed. Then, 10 percent by weight of phenol resin, serving as a binder, was added to and sufficiently mixed with titanium boride powder of 0.3 μm in mean particle diameter. This mixture was continuously extruded and bonded to the periphery of the copper wire

which was degreased and washed. Thus, a titanium boride coating layer of 1  $\mu\text{m}$  in thickness was formed. Then, an inert gas or a reducing gas was sprayed onto this wire, which in turn was covered with a nickel tape of 0.3 mm in thickness. After a seam of this tape was welded, the wire was clad and drawn by squeezing into a wire of 1.0 mm in diameter.

The so produced wire exhibited an electrical conductivity, which can be called an initial conductivity, of 83% at room temperature in accordance with the International Annealed Copper Standard (IACS).

This wire exhibited a conductivity, which can be called a heat-resistant operating conductivity, of 82% in accordance with IACS (International Annealed Copper Standard) after the same was maintained at a temperature of 500° C. for 2000 hour. The nickel layer of this wire was partially oxidized during the exposure to heat.

#### EXAMPLE 2

The surface of the nickel layer provided on the wire which was prepared in Example 1 was further coated with an  $\text{SiO}_2$  ceramics layer of 3  $\mu\text{m}$  in thickness. This wire exhibited an electrical conductivity of 83%. Further, the wire exhibited the same conductivity of 83% IACS, after the same was maintained at a temperature of 500° C. for 2000 hours. No oxidation was noted on this wire.

#### Comparative Example

For the purpose of comparison, a nickel-plated copper wire of 1.0 mm in wire diameter, being coated with a nickel plating layer of 10  $\mu\text{m}$  in thickness, was subjected to a measurement of conductivity, which was 92% IACS. The conductivity was reduced to 65% IACS after the nickel-plated copper wire was maintained at a temperature of 500° C. for 2000 hours. The nickel plating layer provided on the surface of this wire was oxidized during the heat exposure.

As hereinabove described, the composite conductor according to the present invention has an excellent conductivity property and can be manufactured at a low cost, since its core is made of copper or a copper alloy. Further, a conductive ceramics layer provided between the nickel layer and the core prevents interdiffusion even under a high temperature. Further, the conductive ceramics layer minimizes any reduction in conductivity. In addition, the conductive ceramics layer contributes to attaining a high conductivity. Thus, the composite conductor according to the present invention is useful as a conductor for a heat-resistant insulated wire.

Although the present invention has been described and illustrated in detail, it is clearly understood that the same is by way of illustration and example only and is not to be taken by way of limitation, the spirit and scope of the present invention being limited only by the terms of the appended claims.

What is claimed is:

1. A method of manufacturing a composite conductor comprising the following steps:
  - (a) preparing a core material substantially made of copper or a copper alloy;
  - (b) coating said core material by extruding a mixture of electrically conductive ceramics powder and a binder around said core material for forming a conductive ceramics layer around said core material;
  - (c) covering said core material coated with said conductive ceramics layer with a nickel tape under a gas atmosphere selected from the group consisting of inert gases and reducing gases, wherein said tape has a seam;
  - (d) continuously welding said seam;
  - (e) cladding said tape covered, ceramics-coated core material by passing it through a cladding die; and
  - (f) drawing said clad, tape-covered, ceramics-coated core material to form said conductor with a preselected wire diameter.
2. The method of claim 1, further comprising a step of forming a ceramics layer around said conductor.
3. The method of claim 1, wherein said binder substantially consists of a material selected from the group consisting of phenol resin and organometallic polymers.
4. The method of claim 1, further comprising a step of preparing said mixture of electrically conductive ceramics powder by mixing said binder with a ceramics powder material selected from the group consisting of carbides, nitrides, borides and silicides of transition metals, carbon and molybdenum disulfide.
5. The method of claim 4, wherein said ceramics powder material is selected from the group consisting of tungsten carbide, zirconium nitride, titanium boride, molybdenum silicide, carbon and molybdenum disulfide.
6. The method of claim 5, wherein said ceramics powder material is selected from the group consisting of titanium boride and carbon.
7. The method of claim 4, wherein said ceramics powder material comprises particles not more than 5  $\mu\text{m}$  in mean particle diameter.

\* \* \* \* \*